# EUROPEAN PATENT SPECIFICATION

(11) **EP 0 179 555 B1**
(45) Date of publication and mention of the grant of the patent: **23.03.1988**
(21) Application number: 85306175.2
(22) Date of filing: 30.08.1985
(51) Int. Cl.: G03C 5/16, G03C 1/76, G03C 1/84

(54) **Photographic elements sensitive to near infrared**
Zum Nah-Infrarot empfindliche photographische Elemente
Eléments photographiques sensibles à l'infra-rouge proche

(30) Priority: 31.08.1984 GB 8422069
(43) Date of publication of application: 30.04.1986
(73) Proprietor: MINNESOTA MINING AND MANUFACTURING COMPANY, St. Paul, Minnesota 55101 (US)
(72) Inventor: Grzeskowiak, Nicholas E., Harlow Essex CM19 5AE (GB); Philip, James B., Jr. c/o Minnesota Mining, St. Paul Minnesota 55133 (US)
(74) Representative: Bowman, Paul Alan

(56) References cited:
- EP-A- 0 075 231
- FR-A- 1 209 918
- FR-A- 1 527 270
- FR-A- 2 101 859
- FR-A- 2 308 128
- FR-A- 2 357 929
- FR-A- 2 467 421
- US-A- 2 391 127
- US-A- 3 523 022
- US-A- 4 028 104
- US-A- 4 172 731
- APPLIED OPTICS, vol. 20, no. 14, 15th July 1981, pages 2574-2584, New York, US; D.NAOR et al.: "Infrared laser photography with silver-halide emulsion"
- CHEMICAL ABSTRACTS, vol. 79, no. 24, 17th December 1973, page 307, no. 141494g, Columbus, Ohio, US; Z.A.ZAGORSKAYA: "High-resolution photographic emulsion for recording volume holograms" & OPT.-MEKH. PROM. 1973, 40(2), 72

## Description

### Field of the Invention

This invention relates to photographic elements sensitive to light emitted in the near-infrared portion of the spectrum, from 750 nm and above, especially 750 to 1500 nm, and in particular to photographic elements adapted to provide a high quality recording medium for laser diode scanning systems.

### Background of the Invention

A widely used image processing technique is to convert a visible image into electronic data by encoding the brightness of adjacent small areas of the visible image. Such electronic encoding is advantageous for manipulation, transmission and storage of images. It is known to reconvert electronic data into visible images by means of a so-called "scanner system" whereby a finely focussed beam of light is rapidly scanned across a light sensitive medium in a succession of abutting raster lines, whilst modulating the intensity of light so as to reproduce the required image densities, based on the electronic signals.

Lasers, especially those using argon, krypton, helium-neon or helium-cadmium mixtures as the gas lasing media, have been used as sources of high intensity light for this imaging technique. However, the lasers all suffer the disadvantage of requiring an additional, complex device to modulate the intensity of light emitted, and to a greater or lesser extent, from large physical bulk, mechanical fragility and expense of manufacture.

Semiconductor laser diodes are potentially highly suitable as light sources for scanner systems in that their light output can be directly modulated by the electrical signal input, and that they are very compact and physically durable.

However, at present the only commercially available laser diode devices to have acceptably long operational life-times, and be capable of cheap manufacture, are those emitting light in the near-infrared (NIR) portion of the spectrum, from 750 to 1500 nm. Accordingly, in order to utilize laser diode scanner systems for imaging purposes it is necessary to provide a recording medium which is sensitive to light in the NIR range.

It is known to spectrally sensitise photographic silver halide emulsions to near-infrared light, using long chain cyanine dyes, see, for example, Mees and James, The Theory of the Photographic Process, 3rd Edition, MacMillan, 1966, pp. 198-201 and references cited therein.

It has been found that NIR sensitised photographic films, especially those having silver halide grains of mean diameter less than 0.4 um, when supported by the edges in a glassless holder, to prevent contact with other surfaces, and given a uniform overall exposure from a laser diode scanner system emitting at 820 nm, produce images covered with broad swirling interference patterns, referred to hereinafter as "non-contact scanner fringes". These fringes are believed to arise as a result of the reflection of the exposing light from the two interfaces of the film element with surrounding air. The path difference between the rays reflected from the top surface of the film and the bottom surface is controlled by the thickness of the film at a given point, and the net phase diference causes either destructive or constructive interference, causing either diminished or increased exposure to be transmitted into the light sensitive emulsion layer at that given point. The fringes therefore follow contours of microscopic thickness variation in the film element itself, and cover the whole of the image area with broad lines usually about 1 mm apart and often several centimetres in length.

Non-contact interference fringes have not previously been reported in the literature in relation to silver halide emulsion materials. This phenomenon does not occur under the normal conditions of exposure with visible light because the turbidity of the photosensitive emulsion layer is sufficient to scatter the reflections from the back of the film element. However, because of its longer wavelength, infrared light is able to pass without serious scattering through small-grained photographic emulsions, and the coherence of the laser diode output enhances the tendency to form interference patterns. Thus, a photographic emulsion having silver halide grains of mean diameter 0.28um, with a coating weight of silver of 3 g/m², shows detectable fringes. Lowering the grain size to 0.23 um or reducing the coating weight causes more noticeable patterns, whilst emulsions of mean grain diameter 0.20 um or less exhibit severe fringes after non-contact laser diode scanning.

Non-contact scanner fringes seriously degrade the quality of scanner images, especially those having continuous tone gradation. They are not only aesthetically displeasing but they also obscure important information conveyed by small density differences in the image. It is desirable to be able to use photographic emulsions having grains of mean diameter less than 0.4 um preferably less than 0.30 um. Fine grain emulsions having a grain size of 0.4 um or less are advantageous in permitting high spatial resolution, and in having high covering power, permitting a lower coating weight of silver to produce a given maximum optical density after development. Accordingly, photographic elements for use with laser diode scanning systems must be capable of suppressing non-contact interference fringes.

The phenomenon of interference fringes is not unknown in optical recording systems. When exposing shiny surfaced photographic films in contact with other shiny surfaces, e.g. glass supports, dot screens or contact printing negatives, a common problem is the occurrence in the developed image of closely spaced concentric fringe patterns, known as "Newton's rings", see, Encyclopedic Dictionary of Physics, J. Thewlis, Ed., Pergamon, London, 1961, p. 878. These fringes arise due to optical interference between reflections from the top surface of the film and the bottom surface of the contacting support; the size of the local air gap determines the path difference between these two sets of rays, and hence whether their phase difference gives rise to a light or dark fringe causing additional or diminished exposure to be transmitted into the emulsion layer. Newton's rings tend to form isolated areas of pattern, radiating concentrically from the points of contact during exposure, with a narrow fringe spacing which becomes progressively smaller towards the edge of each pattern. These are quite different in appearance to the broad swirling non-contact scanner fringes which cover the whole image area with broad lines usually about 1 mm apart and often several centimetres in length.

Methods are known in the art to prevent formation of Newton's rings. For example, it is known to incorporate matting particles in the outer surface of films. Examples of known matting particles include silica, poly-methyl methacrylate (PMMA), other polyvinyl compounds including copolymers, starch or inorganic salts. The density of matting coverage varies from a relatively small number (e.g. applied at less than 0.1 g/m²) of fairly large particles usually 5 to 10 µm in diameter as disclosed in United States Patent Specification Nos. 4 235 959, 4 022 622, 3 754 924 and 2 322 037, to a particle weight of greater than up to 1 g/m² or 50% of the topcoat binders as disclosed in British Patent Specification Nos. 2 077 935 and 2 033 596 and United States Patent Specification Nos. 3 507 678 and 2 992 101 utilizing smaller particle sizes.

Use of visible laser light as illumination for contact screen exposure of both emulsions produces particularly severe Newton's rings fringes. United States Patent Specification No. 4 343 873 discloses a photographic element designed to minimise such fringes which includes a light-scattering layer through which the light-sensitive layer is exposed to laser light. The light-scattering particles have a diameter of from 50 to 150% of the wavelength of the illuminating laser. The light scattering layer may be coated as an outer layer on the photographic element or beneath other layers.

It is also known to use matting agents in photographic elements for non-optical properties, such as resistance to adhesion, abrasion resistance, retouchability, good draw-down in vacuum frames, and reduced static effects. An example of the use of a matting agent is an infrared sensitive film is disclosed in United States Patent Specification No. 4 266 010 which describes an emulsion topcoat containing PMMA of size in the range 0.2 to 10 pm in an acid-processed gelatin binder, stating this to be suitable for all types of photographic materials including infrared films. A further example is disclosed in United States Patent Specification No. 3 695 888 which describes a photographic emulsion sensitised to infrared light by cyanine dyes with mesoalkylamino substituents and specific supersensitisers, stating that such elements can contain matting agents such as starch, titanium dioxide, zinc oxide, silica, polymeric beads, including 1 to 4 µm beads of a methacrylic acid-methyl methacrylate copolymer disclosed in United States Patent Specification No. 2 992 101 and 1 to 20 ¡.Lm poly-methyl methacrylate beads formed by emulsion polymerisation as disclosed in United States Patent Specification No. 2 701 245.

It has been found that the known types of layers used on photographic elements for suppressing Newton's rings do not prevent the formation of non-contact interference fringes for photographic elements having a photographic emulsion of fine grain size sensitised to the near-infrared.

### Brief Description of the Invention

According to the present invention there is provided a photographic element comprising a support transparent to near infrared radiation above 750 nm, generally in the range 750 to 1500 nm, one or more layers of a silver halide emulsion having grains of an average diameter of not more than 0.4 pm, sensitised to near infrared radiation, characterised in that the element comprises one or more of:
(i) a topcoat layer which is an outermost layer on the same side of the support as the photosensitive emulsion which topcoat layer is a diffuse transmitting layer with respect to near infrared radiation,
(ii) a backing layer which is an outermost layer on the side of the support remote from the photosensitive emulsion which backing layer is a diffuse reflecting layer or absorbing layer with respect to near infrared radiation,
(iii) a subbing layer which is positioned between the support and the photosensitive emulsion which subbing layer is a diffuse transmitting or absorbing layer with respect to near infrared radiation.

A photographic element in accordance with the invention is resistant to the formation of internal optical interference patterns which cause unprotected fine grain near-infrared films to become covered in broad swirling fringes when processed after scanning with a laser diode NIR light source, despite non-contact of the film with other surfaces during exposure.

Three main techniques have been found for preventing formation of non-contact interference fringes, which techniques may be used alone or in combination.

It has been found that the microscopic surface roughness of the element can play an important part in inhibiting the formation of interference fringes. A microscopic surface roughness having 200,000 protrusions per square millimetre provides a marked reduction in the formation of interference fringes and a surface roughness on the backside of the film having 250,000 protrusions per square millimetre will substantially completely eliminate interference fringes, as will a surface roughness of more than 250,000, preferably, 450,000 protrusions per square millimetre on the top surface.

A second technique of inhibiting the formation of interference fringes is to provide a backing or subbing layer containing a dye absorbing light in the wavelength range of the exposing source. When such a layer is used alone as fringe suppression layers of the invention means the layer should have a peak transmission optical density of at least 0.75; when such a layer is used in combination with other fringe suppression means an optical density of at least 0.3 will make a significant contribution to the fringe reduction.

The third technique for reducing fringe formation employs a backing and/or topcoat layer comprising a binder containing particles having a high refractive index substantially preferably greater than 0.3 larger than that of the binder, e.g., desensitised silver halide particles in gelatin.

The use of silver halide particles is advantageous as the halide may be removed during the processing of the photographic element. The high refractive index layer may desirably be removed subsequent to exposure, such as by applying a solvent for the binder.

It has been found that there are several constructions of fine grain near-infrared sensitive photographic elements which will substantially completely suppress the formation of non-contact interference fringes. For example, non-contact interference fringes may be suppressed in such photographic elements incorporating one or more of the methods in the following constructions:
(1) A backing layer on the side of the film base remote from the photosensitive emulsion, comprising a binder containing a surface roughening agent having average particle size not more than 2 µm, generally in the range 0.1 to 2 pm and preferably 0.2 to 2 pm, this outer backing layer having a microscopic roughness of the outer surface, such that each square millimetre of that surface contains at least 250,000 particles which protrude above the average level of that surface by at least 30% of their individual diameters, or by 0.2 um, whichever is less.
(2) A topcoat layer on the same side of the film base as the photosensitive emulsion, comprising a binder containing a surface roughening agent having average particle size not more than 1.5 pm, generally in the range 0.1 to 1.5 µm, and preferably 0.2 to 1.5 µm, this topcoat layer having a microscopic roughness of the outer surface, such that each square millimetre of that surface contains at least 250,000 preferably at least 450,000 particles which protrude above the average level of that surface by at least 30% of their individual diameters, or by 0.2 um, whichever is less.
(3) A backing or subbing layer containing an antihalation dye absorbing light above 750 nm, preferably in the wavelength range 750 to 1500 nm and having a peak transmission optical density of at least 0.75, in that region.
(4) An outermost backing layer containng an antihalation dye giving a peak transmission optical density of at least 0.3 with respect to light above 750 nm, preferably in the wavelength range 750 to 1500 nm, and containing a surface roughening agent of average particle size not more than 2 um, generally in the range 0.1 to 2 pm, and preferably 0.2 to 2 um, this layer having a microscopic roughness of the outer surface such that each square millimetre of that surface contains at least 200,000 particles which protrude above the average level of that surface by at least 30% of their individual diameters, or by 0.2 µm whichever is less, this layer optionally being divided into two separate layers, an outermost backing layer containing the surface roughening agent and the inner backing layer containing the antihalation dye.
(5) The combination of a backing layer having a peak transmission optical density of at least 0.3 with respect to light above 750 nm, preferably in the wavelength range 750 to 1500 nm, and an outermost topcoat layer containing a surface roughening agent having an average particle size not more than 2 µm, generally in the range 0.1 to 2 pm, and preferably 0.2 to 2 pm, this layer having a microscopic roughness of the outer surface such that each square millimetre of that surface contains at least 200,000 particles which protrude above the average level of that surface by at least 30% of their individual diameters, or by 0.2 µm, whichever is less.
(6) The combination of an antihalation layer having a peak transmission optical density of at least 0.3 with respect to light above 750 nm, preferably in the wavelength range 750 to 1500 nm, positioned between the photosensitive layer and the base, and an outermost backing layer or topcoat layer containing a surface roughening agent having an average particle size not more than 2 pm, generally in the range 0.1 to 2 pm, and preferably between 0.1 to 2 pm, this layer having a microscopic roughness of the outer surface such that each square millimetre of that surface contains at least 200,000 particles which protrude above the average level of that surface by at least 30% of their diameters, or by 0.2 µm, whichever is less.
(7) A topcoat layer containing a surface roughening agent having an average particle size not more than 2 um generally in the range 0.1 to 2 um add preferably between 0.2 to 2 pm, this layer having a microscopic roughness of the outer surface such that each square millimetre of that surface contains at least 200,000 particles which protrude above the average level of that surface by at least 30% of their individual diameters, or by 0.2 µm, whichever is less, in combination with an outermost backing layer containing a surface roughening agent having an average particle size not more than 2 um generally in the range 0.1 to 2 µm and preferably between 0.2 to 2 µm, this layer having a microscopic roughness of the outer surface such that each square millimetre of that surface contains at least 200,000 particles which protrude above the average level of that surface by at least 30% of their individual diameters, or by 0.2 µm, whichever is less, and optionally a layer positioned between the backing layer and the support containing an antihalation dye providing a peak transmission optical density of at least 0.3 with respect to light above 750 nm, preferably in the wavelength range 750 to 1500 nm.
(8) A backing and/or topcoat layer comprising a binder containing particles having a refractive index substantially larger than that of the binder (e.g. non-sensitised silver halide particles) said particles having an average particle size below 5 pm and preferably 0.2 to 3 pm, the layer being removable during photographic processing.

It has been found that the microscopic roughness of the photographic element markedly affects the propensity of the element to form non-contact interference fringes when imaged with a scanning laser. In particular, it has been found that the provision of an outer backing layer providing a microscopic roughness having at least 250,000 protrusions per square millimetre above the average level of the surface will prevent fringe formation, assuming irradiation takes place from the other side of the element. Similarly, fringe formation can be prevented by provision of a topcoat layer the microscopic surface roughness providing at least 250,000 preferably 450,000 protrusions per square millimetre assuming the element is irradiated from the same side as this layer. This microscopic surface roughness is significantly different from that found in prior art photographic elements incorporating layers of matting agents; in general matting layers in the prior art tend to provide surfaces with less than half the number of protrusions than those required in the present invention and often contain less than one tenth of the number of protrusions than the surfaces used in the invention.

It is possible to substantially suppress fringe formation by employing a backing or subbing layer incorporating an antihalation dye to provide a peak transmission optical density of at least 0.75 in the range 750 to 1500 nm.

Combinations of surface roughening layers and antihalation layers may be employed as described above in which case the critical parameters of surface roughening and optical density for each individual layer may be reduced compared to that required when such layers are used as the only means for reducing fringe formation since the effect of the combination of layers is additive. It has been found that a suitable microscopic surface roughness for an outer layer to be used in combination with a further fringe suppressing layer is 200,000 protrusions per square millimetre. The optical density required by an antihalation layer to be used in combination with a surface roughening layer is at least 0.3.

Particle-containing surface layers described above are preferably used on the back surfaces of the elements, or on both outermost surfaces, rather than as topcoats on the photosenstive emulsion side only, since, surprisingly, the suppression of non-contact laser scanner fringes by surface roughened backings is superior to that by similar topcoats on the emulsion side assuming the exposure is from the emulsion side.

Advantageous surface roughening agents for use in such layers are particles of organic polymers, particularly of polymethyl methacrylate or developer-soluble polymers such as methacrylic acid- methacrylic ester copolymers, e.g. as described in United States Patent Specification No. 2 992 101. Other suitable organic polymers, when used in the particle size range, and loading needed to give the matting properties specified above, are other polyvinyl compounds or vinyl compound copolymers, e.g. as described in British Patent Specification Nos. 2 078 992 and 2 033 596 and United States Patent Specification Nos. 4 287 299 and 3 079 257. Other suitable materials include silicaa or composites of silica with polymer, e.g. as described in United States Patent Specification Nos. 4 235 959, 3 920 456, 3 591 379 and 3 222 037, hardened gelatin, water soluble inorganic salts, or starch, dextran and mixtures of these polymers, as described in British Patent Specification No. 2 077 935.

One type of matting agent known in the art consists of very small particles of silica, typically of diameter 0.1 um or less. On dispersion in coating binders such as aqueous gelatine, these small particles form tightly-bound aggregates, typically of 1 pm or greater in diameter, which behave as though they were a single particle. The matting properties required for the purposes of this invention may be obtained either by the use of single particles in the required size range, or equally by use of aggregates, the overall size of which falls in the same required range.

Suitable materials of high refractive index include non-photosensitive silver halide crystals, which are readily produced in uniform sizes and removed by photographic fixers. Silver halides generally have a refractive index in the range 2.0 to 2.2. Other suitable materials of high refractive index include zinc oxide and calcium carbonate.

Gelatin is a suitable binder for all these layers and has a refractive index of about 1.5.

When small polymer or other particles, especially those of mean diameter 1 ¡.Lm or below, are used to matt the surface of a layer of binder as this is coated, the height of the protrusions above the average surface level, and the number of particles protruding, is dependent not only on the weight of paticles contained in the layer, but also on the coating and drying conditions used. It is important to select conditions for coating and drying which give the high degree of particle protrusion required by this invention and these parameters will be appreciated by a person skilled in the art. One technique which has proved to provide satisfactory surface roughness when used with suitable formulations is to pass the wet element immediately after coating into a chill zone at 13°C at 30% relative humidity to cause the gel to set and thereafter to dry at 30°C, at 30% relative humidity. It was found that the thin layers were dry in 30 seconds to 1 minute.

In addition to the above matting particles introduced for the purposes of surface roughening in accordance with the invention, the photographic element can contain small quantities (less than 0.1 g/m²) of larger polymer, silica or other matting agent with particles of mean diameter 5 pm and greater, to improve mechanical properties such as adhesion and abrasion resistance.

Silver halide emulsions useful in the photographic elements of this invention may comprise silver bromide, silver chloride, silver chlorobromide silver bromoiodide or silver chlorobromiodide, and can be prepared by any of the well known procedures, e.g. as described in Research Disclosure 17643, December 1978, par. II and III. The emulsions have a particle size of not more than 0.4 um, generally in the range 0.05 to 0.4 pm.

The emulsions can be sensitised to near-infrared using the dyes disclosed in European Patent Application Publication No. 0 088 595, or using any of the other spectral sensitising dyes known in the art to give sensitivity to radiation of wavelength 750 to 1500 nm, preferably 750 to 900 nm, e.g. as described in Mees and James, The Theory of the Photographic Process, 3rd Ed., pp. 198-199.

Silver halide emulsions present in the photographic element of this invention can be protected against the production of fog and can be stabilised against loss of sensitivity during keeping. Suitable antifoggants and stabilisers are described, for example, in Research Disclosure 17643, December 1978, par. VI.

Silver halide emulsions present in the photographic elements of this invention can employ optical brightening agents as described, for example, in Research Disclosure 17643, December 1978, par. V.

The spectrally sensitised silver halide emulsions used in the invention can contain speed increasing compounds, e.g. those described in Research Disclosure 17643, December 1978, par. XXI.

The layers of the photographic elements can contain various colloids as vehicles or binding agents, e.g. those described in Research Disclosure 17643, December 1978, par. IX. Such colloids can be hardened by various organic and inorganic hardeners, e.g. those described in Research Disclosure 17643, December 1978, par. X.

The photographic elements of the invention can contain antistatic or conducting layers, plasticisers and lubricants, surfactants, as described, for example, in Research Disclosure 17643, December 1978, par. XI, XII and XIII.

Photographic emulsions used in the invention can be coated on a wide variety pftransparentsupports, e.g. those described in Research Disclosure 17643, December 1978, par. XVIII.

The sensitising dyes and other emulsion addenda can be incorporated into the layers of the photographic elements by various methods known in the photographic elements by various methods known in the art, e.g. those described in Research Disclosure 17643, December 1978, par. XIV. Similarly the photographic elements can be coated on photographic supports by various procedures. Supports and coating procedures are described, for example, in Research Disclosure 17643, December 1978, par. XVV and XVII.

The sensitised silver halide emulsions used in this invention can be processed after exposure to form a visible silver and/or dye image by associating the silver halide with an aqueous alkaline medium in the presence of a developing agent as described, for example, in Research Disclosure 17643, December 1978, par. XIX.

Whilst the invention is described in detail for elements containing silver halide grains below 0.4 pm in diameter; the methods for fringe suppression are equally applicable to elements containing other photosensitive silver halide crystals which may permit formation of scanner fringes due to low turbidity. In particular the invention is applicable to elements containing tabular grains of silver halide exceeding 0.4 um in diameter, but of high aspect ratio, especially if these are present as a low overall fraction of the silver halide grains in the element, the remainder being comprised of fine grains.

The photographic elements of this invention can be useful in physical development systems, image transfer systems, dry development systems, diffusion transfer systems, printing and lithography, print-out and direct-print systems as, described, for example, in Research Disclosure 17643, December 1978, par. XXII, XXIII, XXIV, XXV, XXVI and XXVII. The invention will now be illustrated by the following Examples.

In the Examples the evaluation of the samples was conducted as follows:
Evaluation of Samples by Non-contact Laser Diode Scanning, and Measurement of Fringes

Samples were evaluated by uniform exposure in a scanner system in which the radiation from a Hitachi HLP 1400 laser diode emitting at 815 nm was focused to a circular spot of 50 um diameter on the surface of the sample. The focused spot was scanned in raster pattern of 200 lines/cm over the sample by means of an oscillating galvanometer mirror in path of the infrared beam. The intensity of the exposure was increased stepwise to produce after processing a scale from minimum to maximum density on the sample. The samples were then developed using an automatic roller processor 3M type XP507 utilising Eastman Kodak RP X-Omat processing solutions. A visual inspection for fringe patterns was made, and these assessed using the following ranking order:
1 No fringes seen
2 Almost undetectable fringes
3 Very faint, seen only under close scrutiny
4 Diffuse patterns
5 Faint, but sharply defined fringes
6 Readily noticed fringes
7 Sharply defined fringe patterns.

The fringe patterns were quantitatively evaluated by tracing with a Joyce-Loebl MDM6 microdensitometer using a small (2.0 x 0.25 mm) slit aperture. The maximum transmission optical density difference (O.D.) thus measured between light and dark fringes is given in the Examples. The O.D. was measured in areas scanned to mean optical density of between 1.0 and 2.0, in which region the emulsion had contrast values of from 2.5 to 3.5.

The measurement of surface reflectivity of the samples in the Examples was conducted as follows:
Measure of direct (specular) surface reflectivity of matted back surfaces

Samples were prepared prior to testing by physical removal of the photosensitive emulsion layer, and by application of a densely I.R. absorbing, non-reflective layer in its place. The untreated side of the samples was then irradiated at an angle of 10° to the normal with a collimated beam of known energy, of 5 mm diameter, from a laser diode emitting at 815 nm. A radiometric detector was used to monitor the reflected energy at a total angle of 20° to the incident beam (Optronics model 730A). This detector was sited at a distance of 30 cm from the test surface, and admitted light through a circular aperture of 1 cm diameter.

As the same detector was used to assess both incident and reflected energy, a simple calculation allowed percentage reflectivity to be ascertained. Care was taken with choice of laser diode/sample film/ detector configurations to ensure that any extraneous energy was omitted from measurements.

The examination of matted surfaces of the samples in the Examples was conducted as follows:
Scanning electron microscope examination of matted surfaces (S.E.M.)

A sample (approximately 1 cm²) of the film was bonded to a pin stub, with the surface to be examined uppermost. A gold coating, approximately 25 nm thick, was applied, using an International Scientific Instruments Inc. (ISI) PS-2 coating unit, at 1.2 kVand 10 mA for 2 minutes. The samples were examined in an ISI Super IIIA scanning electron microscope, operating at 10 kV. The samples were angled at +20°. In each case a photograph was taken at a print magnification of 5000X, using an internal calibration marker. Particle counts were made within a grid representing an area of 10 um x 10 µm. Particles were counted if they appeared to extend above the average surface level by at least 30% of their diameter, or 0.2 um, whichever was smaller. In samples where only large, infrequent particles were present, photographs at 2000X or lower magnification were taken, and counts made over a more extensive area.

The results reported are an average of counts made from photographs of. two different parts of each surface examined.

### Example 1

### Preparation of NIRsensitive silver halide emulsions and their use in photographic elements for laser diode scanner tests

An emulsion containing 64% silver chloride moles and 36% silver bromide moles with cubic grains having an average grain size of 0.28 um and a narrow distribution curve was prepared by a double jet precipitation method described in Example 17B of European Patent Application Publication No. 0 088 595.

Similar emulsions having mean grain sizes of 0.23 µm, 0.20 pm, 0.16 µm and 0.13 pm were likewise prepared, using successively lower temperatures for precipitation. All these emulsions were conventionally gold and sulphur sensitised and stabilised, and NIR spectral sensitising dye, triphenylphosphine supersensitiser, wetting agents and hardener were added as described in the basic formulation in Example 18 of European Patent Application Publication No. 0 088 595. The emulsions were coated individually on transparent 0.18 mm subbed polyester base, to give 2.7 to 3.0 g/m² silver coating weight. A supercoat of 200 ml of 5% aqueous gelatin containing 100 mg Superamide L9C and 0.15 ml Teepol 610 wetting agents and 4.5 ml of 2% solution of formaldehyde hardener, but no matting agents or filter dyes, was simultaneously applied to give a top layer of 1.33 g/m² gelatin. The back surface of the film base was left uncoated. Superamide L9C is a high activity lauric acid-diethanolamine condensate commercially available from Millmaster-Onyx UK. Teepol 610 is a sodium salt of a secondary alkyl sulphate commercially available from Shell Chemicals UK Ltd.

The samples were evaluated as described above and the results shown in Table 1.

This Example demonstrates the increasing severity of scanner fringes with decreasing silver halide grain size.

### Example 2

### Photographic elements according to the invention having backing layers containing PMMA particles, and resistant to scanner fringes

Emulsions were prepared, NIR sensitised and coated as in Example 1, but using an 0.18 mm subbed polyester base provided with a backing layer containing 0.3 g/m² of poly(methyl methacrylate) particles of mean diameter 0.5 pm in a gelatin binder (1.3 g/m²), which was coated from an aqueous solution also containing as in Example 1 Superamide L9C and Teepol 610 wetting agents, and formaldehyde hardener. Immediately after coating onto the film base, the wet backing layer was passed briefly through a chill zone, at 13°C and 30% relative humidity, causing the gel to set, drying was then brought about at 30°C and 30% relative humidity, and appeared to be complete within 1 minute. The samples were tested in the laser diode scanner system as described above and the results reported in Table 2.

The coatings of the same grain size emulsions in Example 1 act as control standards.

### Example 3

### Photographic elements according to the invention having backing layers containing non-photosensitive silver halide grains

An 0.16 µm chlorobromide emulsion was coated as in Example 1, but using a 0.18 mm polyester base provided with a backing layer containing silver halide grains, insensitive to NIR light, in a gelatin binder (1.3 g/m²). The effect on scanner fringes of different sizes and loadings of backing grains is reported in Table 3.

### Example 4

### Photographic element having backing layer containing other surface roughening agents

A 0.16 um chlorobromide emulsion was coated as in Example 1, but on a 0.18 mm subbed polyester base having a backing containing particles (mean grain size of 0.5 to 2.0 pm) of alkali-soluble methacrylic acid-ethyl methacrylate copolymer, in a gelatin binder (1.3 g/m²), which was coated from an aqueous solution containing as in example 1 Superamide L9C or Teepol 610 wetting agents, and formaldehyde hardener as in Example 1. An otherwise identical sample was prepared in which the polymer particles were replaced by a lower loading of silica particles of mean diameter 5 um. These samples were tested in comparison with an unbacked one, and the results are reported in Table 4.

### Example 5

### Effect of antihalation backing on scanner fringes (0.16 µm chlorobromide emulsion)

A 0.16 um chlorobromide emulsion was coated as in Example 1, but on a 0.18 mm subbed polyester base having a backing consisting of gelatin 5 g/m², containing an antihalation dye absorbing strongly between 750 and 900 nm, (Dye 29 in European Patent Application Publication No. 0 01 646) with an optical density of 0.40 at 820 nm.This was tested in comparison with an unbacked sampled in the laser diode scanner system, and the results are reported in Table 5.

### Example 6

### Use of iodobromide emulsions

A 3% iodobromide emulsion of average grain size 0.21 um was prepared, chemically sensitized, stabilised, spectrally sensitised, and coated on transparent 0.18 mm subbed polyester base, in accordance with Example 17A of European Patent Application Publication No 0 088 595. A topcoat of 1.3 g/m² of gelatin was simultaneously applied.

Similar coatings were made on 0.18 mm polyester based having an antihalation backing consisting of up to three consecutive layers of gelatin (5 g/m²) containing a dye (Dye 29 in European Patent Application No 0 101 646), absorbing strongly between 750 and 900 nm, giving overall optical densities of 0.45,0.8 and 1.2 at 820 nm. These coatings were tested in the laser diode scanner system, and the results reported in Table 5

The antihalation layers clearly aid the suppression of fringes.

### Example 7

### Relation of scanner fringe formation to surface specular reflectivity and surface roughness

A 0.16 µm chlorobromide emulsion was coated as in Example 1, but using 0.18 µm subbed polyester bases provided with backing layers containing a series of concentrations of PMMA particles of mean diameter 0.5 pm, coated in a gelatin binder (1.3 g/m²) as in Example 2. These samples were tested in a laser diode scanner system and the effect on fringe formation is reported in Table 6.

### Example 8

### Coatings with both dye antihalo and PMMA particle cover

### (a) Antihalation Dye and Conventional Matting Agents only

A chlorobromide emulsion of grain size 0.26 um was prepared and sensitized using the methods of Example 1. The emulsion was coated on a 0.18mm polyester base, at 2.4 g/m² silver coverage, simultaneously applying a thin gelatin (1.3 g/m²) topcoat containing 0.036 g/m² of PMMA particles of 2.5 µm mean diameter. The opposite side of the base was provided with a layer of gelatin (5 g/m²) containing an infrared absorbing dye (Dye 17 in European Patents Application Publication No. 0 101 646) giving an infrared absorption from 750 to 900 nm, with an optical density of 0.6 at 815 nm and having a gelatin topcoat (1.3 g/m²) containing 0.065 g/m² of PMMA particles of 6 µm mean diameter (backing layer). This coating was tested in a laser diode scanner and the result is reported in Table 7.

### (b) Antihalation Dye and Surface Roughening Agents According to the Invention

The coating in (a) was repeated, with the addition of 0.18 g/m² of 0.5 µm PMMA spheres to both the front and the back topcoat layers. The sample was tested in a laser scanner and the result reported in Table 7.

Sample (a) was found to give distinctly visible, non-contact scanner fringes whereas Sample (b) did not give any non-contact scanner fringes under the most stringent conditions a laser diode scanner testing.

### Example 9

### Photographic elements having outer matting layers containing particles of an alkali-soluble copolymer

A 0.16 µm chlorobromide emulsion was coated as in Example 1, but on a 0.18 mm polyester base having a backing containing particles of alkali-soluble methacrylic acid-ethyl methacrylate copolymer, in a gelatin binder (1.3g/m²), which was coated from an aqueous solution containing Superamide L9C and Teepol 610 wetting agents, and formaldehyde hardener as in Example 1. The copolymer particles were of mean diameter 0.75 pm but included a broad range of diameters up to 2 pm. Samples containing different densities of this matting agent were tested for fringe formation in comparison with an unbacked one, and the results are reported in Table 8.

The degree to which fringes are suppressed is dependent on the type of construction, and on the surface density of protruding particles produced by the matting agent. Further coatings were made in a similar manner using the same 0.16 pm chlorobromide emulsion and suspensions of copolymer matting agent, but using a 0.18 mm polyester base having applied to one side an infra-red absorbing antihalation layer, as in Example 5. The matting layers were applied directly over the antihalation layer, and the photosensitive emulsion to the opposite side of the film base.

A third set of coatings has made of the same chlorobromide emulsion on an unbacked 0.18 mm polyester base, as in Example 1, except that the usual emulsion supercoat was replaced by the matting suspensions of copolymer particles as described above.

The coatings housing matting backing over an antihalation layer and those having matting supercoats to the emulsion were also tested in the laser diode scanner, and the results represented in Table 8.

## Claims

1. A photographic element comprising a support transparent to near infrared radiation, one or more layers of a silver halide emulsion having grains of an average diameter of not more than 0.4 µm, sensitized to near infrared radiation, characterised in the element comprises one or more of:
(i) a topcoat layer which is an outermost layer on the same side of the support as the photosensitive emulsion which topcoat layer is a diffuse transmitting layer with respect to near infrared radiation,
(ii) a backing layer which is an outermost layer on the side of the support remote from the photosensitive emulsion which backing layer is a diffuse reflecting layer or absorbing layer with respect to near infrared radiation,
(iii) a subbing layer which is positioned between the support and the photosensitive emulsion which subbing layer is a diffuse transmitting or absorbing layer with respect to near infrared radiation.

2. A photographic element as claimed in Claim 1, characterised in that the element comprises a backing layer, comprising a binder containing a surface roughening agent having average particle size not more than 2 um, the backing layer having a microscopic roughness of the outer surface, such that each square millimetre of that surface contains at least 250,000 particles which protrude above the average level of that surface by at least 30% of their individual diameters, or by 0.2 um, whichever is less.

3. A photographic element as claimed in Claim 1, characterised in that the element comprises a topcoat layer, comprising a binder containing a surface roughening agent having average particle size not more than 2 pm, this topcoat layer having a microscopic roughness of the outer surface, such that each square millimetre of that surface contains at least 250,000 particles which protrude above the average level of that surface by at least 30% of their individual diameters, or by 0.2 pm, whichever is less.

4. A photographic element as claimed in Claim 1, characterised in that the microscopic surface roughness is such that each square millimetre of that surface contains at least 450,000 particles which protrude above the average level of that surface by at least 30% of their individual diameters, or by 0.2 µm, whichever is less.

5. A photographic element as claimed in Claim 1, characterised in that the element comprises a backing or subbing layer containing an antihalation dye absorbing light in the near infrared and having a peak transmission optical density of at least 0.75, in that range.

6. A photographic element as claimed in Claim 1, characterised in that the element comprises a backing layer containing an antihalation dye giving a peak transmission optical density of at least 0.3 with respect to light in the near infrared, and containing a surface roughening agent of average particle size not more than 2 pm, this layer having amicroscopic roughness of the outer surface such that each square millimetre of that surface contains at least 200,000 particles which protrude above the average level of that surface by at least 30% of their individual diameters, or by 0.2 um, whichever is less.

7. A photographic element as claimed in Claim 1, characterised in that the element comprises a backing layer having a peak transmission optical density of at least 0.3 with respect to light in the near infrared, and a topcoat layer containing a surface roughening agent having an average particle size not more than 2 pm, this layer having a microscopic roughness of the outer surface such that each square millimetre of that surface contains at least 200,000 particles which protrude above the average level of that surface by at least 30% of their individual diameters, or by 0.2 pm, whichever is less.

8. A photographic element as claimed in Claim 1, characterised in that the element comprises an antihalation subbing layer having a peak transmission optical density of at least 0.3 with respect to light in the near infrared, and a backing layer or topcoat layer containing a surface roughening agent having an average particle size not more than 2 um, this layer having a microscopic roughness of the outer surface such that each square millimetre of that surface contains at least 200,000 particles which protrude above the average level of that surface by at least 30% of their individual diameters, or by 0.2 pm, whichever is less.

9. A photographic element as claimed in Claim 1, characterised in that the element comprises a topcoat layer containing a surface roughening agent having an average particle size not more than 2 pm, this layer having a microscopic roughness of the outer surface such that each square millimetre of that surface contains at least 200,000 particles which protrude above the average level of that surface by at least 30% of their individual diameters, or by 0.2 pm, whichever is less and a backing layer containing a surface roughening agent having an average particle size not more than 2 pm, this layer having a microscopic roughness of the outer surface such that each square millimetre of that surface contains at least 200,000 particles which protrude above the average level of that surface by at least 30% of their individual diameters, or by 0.2 pm, whichever is less, and optionally a subbing layer containing an antihalation dye providing a peak transmission optical density of at least 0.3 with respect to light in the near infrared.

10. A photographic element as claimed in Claim 1, characterised in that the element comprises a backing and/or topcoat layer comprising a binder containing particles having a refractive index substantially larger than that of the binder having an average particle size below 5 um, the layer(s) being removable during photographic processing.

11. A photographic element as claimed in Claim 10, characterised in that the element is sensitive to radiation on the wavelength range 750 to 900 nm.

12. A photographic element as claimed in any one of Claims 1 to 3 and 5 to 9, characterised in that the particles of roughening agent have an average particle size in the range 0.2 to 2 µm.

13. A photographic element as claimed in any one of Claims 1 to 3, 5 to 9 and 12, characterised in that the roughening agent is selected from poly-methyl methacrylate and copolymers of methacrylic acid with methyl or ethyl methacrylate.

14. A photographic element as claimed in Claim 10, characterised in that the material of high refractive index has an average particle size in the range 0.2 to 3 pm.

15. A photographic element as claimed in Claim 14, characterised in that the material of high refractive index is selected from silver halide, zinc oxide and calcium carbonate.

16. A method of recording an image substantially free of non-contact interference fringes which comprises exposing a photographic element as claimed in any preceding claim in absence of contact with other surfaces with radiation in the near infrared from a laser diode scanning system positioned on the emulsion side of the photographic element and thereafter processing said element to develop the image.

## Patentansprüche

1. Photographisches Aufzeichnungsmaterial, umfassend einen für Strahlung im nahen Infrarot durchlässigen Träger, eine oder mehrere Schichten mit Silberhalogenidemulsionskörnern von einem durchschnittlichen Durchmesser mit nicht mehr als 0,4 µm, sensibilisiert für Strahlung im nahen Infrarot, dadurch gekennzeichnet, daß das Aufzeichnungsmaterial umfaßt:
(i) mindestens eine Oberguß-Schicht, die sich als Aufguß-Schicht auf der gleichen Seite wie die Emulsion befindet, wobei diese Oberguß-Schicht eine diffus durchlässige Schicht bezüglich der Strahlung im nahen Infrarot ist;
(ii) eine Rückschicht, die als Gegenschicht zur photographischen Emulsion auf der Rückseite des Trägers angeordnet ist, wobei die Rückschicht eine Strahlung im nahen Infrarot diffus reflektierende oder absorbierende Schicht ist;
(iii) mindestens eine Substrat-Schicht, die zwischen dem Träger und der lichtempfindlichen Emulsion angeordnet ist, wobei die Substrat-Schicht eine Strahlung im nahen Infrarot diffus durchlässige oder absorbierende Schicht ist.

2. Aufzeichnungsmaterial nach Anspruch 1, dadurch gekennzeichnet, daß das Aufzeichnungsmaterial eine Rückschicht umfaßt, die ein Bindemittel mit einem Mittel zur Aufrauhung der Oberfläche mit einer durchschnittlichen Korngröße von höchstens 2 µm enthält, wobei die Rückschicht eine mikroskopische Oberflächenrauhigkeit aufweist derart, daß jeder Quadratmillimeter dieser Oberfläche mindestens 250 000 Teilchen aufweist, die um mindestens 30% ihres Durchmessers über den Durchschnittswert Oberfläche oder um 0,2 um als Hochstwert herausragen.

3. Aufzeichnungsmaterial nach Anspruch 1, dadurch gekennzeichnet, daß das Aufzeichnungsmaterial eine Oberguß-Schicht umfaßt, die ein Bindemittel mit einem Mittel zur Aufrauhung der Oberfläche mit einer durchschnittlichen Korngröße von höchstens 2 um enthält, wobei die Oberguß-Schicht eine mikroskopische Oberflächenrauhigkeit aufweist derart, daß jeder Quadratmillimeter dieser Oberfläche mindestens 250 000 Teilchen aufweist, die um mindestens 30% ihres Durchmessers über der Durchschnittswert Oberfläche oder um 0,2 um als Hochstwert herausragen.

4. Aufzeichnungsmaterial nach Anspruch 1, dadurch gekennzeichnet, daß die microskopische Oberflächenrauhigkeit derart beschaffen ist, daß jeder Quadratmillimeter dieser Oberfläche mindestens 450 000 Teilchen aufweist, die um mindestens 30% ihres Durchmessers über den Durchschnittswert der Oberfläche oder um 0,2 um als Hochstwert herausragen.

5. Aufzeichnungsmaterial nach Anspruch 1, dadurch gekennzeichnet, daß das Aufzeichnungsmaterial eine Rückschicht oder Substrat-Schicht umfaßt, die einen Lichthoffarbstoff enthält, der eine maximale Dichte der optischen Durchlässigkeit von mindestens 0,75 bezüglich Licht im nahen Infrarot ergibt.

6. Aufzeichnungsmaterial nach Anspruch 1, dadurch gekennzeichnet, daß das Aufzeichnungsmaterial eine Rückschicht umfaßt, die einen Lichthoffarbstoff mit einer maximalen Dichte der optischen Durchlässigkeit von mindestens 0,3 bezüglich Licht im nahen Infrarot und ein Mittel zur Aufrauhung der Oberfläche mit einer durchschnittlichen Korngröße von höchstens 2 µm enthält, wobei diese Rückschicht eine microskopische Oberflächenrauhigkeit aufweist derart, daß jeder Quadratmillimeter dieser Oberfläche mindestens 200 000 Teilchen aufweist, die um mindestens 30% ihres Durchmessers über den Durchschnittswert der Oberfläche oder um 0,2 um als Höchstwert herausragen.

7. Aufzeichnungsmaterial nach Anspruch 1, dadurch gekennzeichnet, daß das Aufzeichnungsmaterial eine Rückschicht die eine maximale Dichte der optischen Durchlässigkeit von mindestens 0,3 bezüglich Licht im nahen Infrarot hat, sowie eine Oberguß-Schicht umfaßt, die ein Mittel zur Aufrauhung der Oberfläche mit einer durchschnittlichen Korngröße von höchstens 2 um enthält, wobei die Oberguß-Schicht eine microskopische Oberflächenrauhigkeit aufweist derart, daß jeder Quadratmillimeter dieser Oberfläche mindestens 200 000 Teilchen aufweist, die um mindestens 30% ihres Durchmessers über den Durchschnittswert der Oberfläche oder um mindestens 0,2 um als Höchstwert herausragen.

8. Aufzeichnungsmaterial nach Anspruch 1, dadurch gekennzeichnet, daß das Aufzeichnungsmaterial eine Lichthofschutzschicht-Substratschicht mit einer maximalen Dichte der optischen Durchlässigkeit von mindestens 0,3 bezüglich Licht im nahen Infrarot sowie eine Rückschicht oder Oberguß-Schicht umfaßt, die ein Mittel zur Aufrauhung der Oberfläche mit einer durchschnittlichen Korngröße von höchstens 2 um enthält, wobei diese Schicht eine microskopische Oberflächenrauhigkeit aufweist derart, daß jeder Quadratmillimeter dieser Oberfläche mindestens 200 000 Teilchen aufweist, die um mindestens 30% ihres Durchmessers über den Durchschnittswert der Oberfläche oder um 0,2 um als Höchstwert herausragen.

9. Aufzeichnungsmaterial nach Anspruch 1, dadurch gekennzeichnet, daß das Aufzeichnungsmaterial eine Oberguß-Schicht mit einem Mittel zur Aufrauhung der Oberfläche mit einer durchschnittlichen Korngröße von höchstens 2 um, wobei die Oberguß-Schicht eine microskopische Oberflächenrauhigkeit aufweist derart, daß jeder Quadratmillimeter dieser Oberfläche mindestens 200 000 Teilchen aufweist, die um mindestens 30% ihres Durchmessers über den Durchschnittswert der Oberfläche oder um 0,2 um als Höchstwert herausragen, sowie eine Rückschicht, die ein Mittel zur Aufrauhung der Oberfläche mit einer durchschnittlichen Korngröße von höchstens 2 um enthalt, wobei die Rückschicht eine microskopische Oberflächenrauhigkeit aufweist derart, daß jeder Quadratmillimeter dieser Oberfläche mindestens 200 000 Teilchen aufweist, die um mindestens 30% ihres Durchmessers über den Durchschnittswert der Oberfläche oder um 0,2 um als Höchstwert herausragen, und gegebenenfalls eine Substrat-Schicht umfaßt, die einen Lichthoffarbstoff mit einer maximalen Dichte der optischen Durchlässigkeit von mindestens 0,3 bezüglich Licht im nahen Infrarot enthält.

10. Aufzeichnungsmaterial nach Anspruch 1, dadurch gekennzeichnet, daß das Aufzeichnungsmaterial eine Rückschicht und/oder Oberguß-Schicht umfaßt, die ein Bindemittel mit Teilchen mit einem Brechungsindex enthält, der wesentlich größer ist als der des Bindemittels, wobei die Teilchen eine durchschnittliche Korngröße unter 5 um haben, und wobei die Schicht bzw. die Schicht während der photographischen Entwicklung entfernbar sind.

11. Aufzeichnungsmaterial nach Anspruch 10, dadurch gekennzeichnet, daß das Aufzeichnungsmaterial gegenüber Strahlung im Wellenlängenbereich von 750 bis 900 nm empfindlich ist.

12. Aufzeichnungsmaterial nach einem der Ansprüche 1 bis 3 und 5 bis 9, dadurch gekennzeichnet, daß die Teilchen des aufrauhenden Mittels ein durchschnittliche Korngröße im Bereich von 0,2 bis 2 um aufweisen.

13. Aufzeichnungsmaterial nach einem der Ansprüche 1 bis 3, 5 bis 9 und 12" dadurch gekennzeichnet, daß das aufrauhende Mittel eine Methylmethacrylat-Polymerisat oder eine Copolymerisat von Methacrylsäure mit Methacrylsäure methyl- oder äthylester ist.

14. Aufzeichnungsmaterial nach Anspruch 10, dadurch gekennzeichnet, daß das Material mit hohem Brechungsindex eine durchschnittliche Korngröße im Bereich von 0,2 bis 3 um hat.

15. Aufzeichnungsmaterial nach Anspruch 14, dadurch gekennzeichnet, daß das Material mit hohem Brechungsindex eine Silberhalogenid, Zinkoxid oder Calciumcarbonat ist.

16. Verfarhren zur Aufzeichnung eines Bildes, das im wesentlichen frei von Nichtkontakt-Interferenzmustern ist, dadurch gekennzeichnet, daß man ein photographisches Aufzeichnungsmaterial nach einem der vorhergehenden Ansprüche ohne Berührung mit anderen Oberflächen in einer Strahlung im nahen Infrarot aus einem Laserdiode-Abtastsystem belichtet, das auf der Emulsionsseite des photographischen Aufzeichnungsmaterials angeordnet ist, und anschließend das Aufzeichnungsmaterial zur Entwicklung des Bildes verarbeitet.

## Revendications

1. Elément photographique comprenant un support transparent au rayonnement proche de l'infrarouge, une ou plusieurs couches d'une émulsion d'halogénure d'argent comportant des grains d'un diamètre moyen non supérieur à 0,4 pm, sensibilisées au rayonnement dans le proche infrarouge caractérisé en ce qu'il comprend une ou plusieurs des couches suivantes:
(i) une couche supérieure qui est une couche externe se situant du même côté du support que l'émulsion photosensible, cette couche supérieure étant une couche de transmission diffuse par rapport au rayonnement dans le proche infrarouge,
(ii) une couche dorsale qui est une couche extérieure se situant du côte du support, opposé à l'émulsion photosensible, cette couche dorsale étant une couche d'absorption ou une couche de réflexion diffuse par rapport au rayonnement dans le proche infrarouge,
(iii) une couche de substrat qui est disposée entre le support et l'émulsion photosensible, cette couche de substrat étant une couche d'absorption ou de transmission diffuse par rapport au rayonnement dans le proche infrarouge.

2. Elément photographique suivant la revendication 1, caractérise en ce qu'il comprend une couche dorsale, comportant un liant contenant un agent de rugosité superficielle d'une taille moyenne de particules non supérieure à 2 um, cette couche dorsale présentant une rugosité microscopique de sa surface externe, de telle sorte que chaque millimètre carré de cette surface contient au moins 250.000 particules qui font saillie au-dessus du niveau moyen de cette surface, suivant au moins 30% de leurs diamètres individuels, ou suivant 0,2 micron, quelle que soit la valeur qui est la moindre.

3. Elément photographique suivant la revendication 1, caractérisé en ce qu'il comprend une couche supérieure, comprenant un liant contenant un agent de rugosité superficielle d'une taille moyenne de particules non supérieure à 2 pm, cette couche suoérieure présentant une rugosité microscopique de sa surface externe, de sorte que chaque millimètre carré de cette surface contient au moins 250.000 particules qui font saillie au-dessus du niveau moyen de cette surface, suivant au moins 30% de leurs diamètres individuels, ou suivant 0,2 pm, quelle que soit la valeur qui est la moindre.

4. Elément photographique suivant la revendication 1, caractérisé en ce que la rugosité superficielle microscopique est telle que chaque millimètre carré de cette surface contient au moins 450.000 particules qui font saillie au-dessus du niveau moyen de cette surface suivant au moins 30% de leurs diamètres individuels, ou suivant 0,2 um, quelle que soit la valeur qui est la moindre.

5. Elément photographique suivant la revendication 1, caractérisé en ce qu'il comprend une couche dorsale ou de substrat, contenant un colorant antihalo absorbant la lumière dans le proche infrarouge et ayant une densité optique de transmission maximale d'au moins 0,75 dans cet intervalle.

6. Elément photographique suivant la revendication 1, caractérisé en ce qu'il comprend une couche dorsale comprenant un colorant antihalo donnant une densité optique de transmission maximale d'au moins 0,3 par rapport à la lumière du proche infrarouge, et contenant un agent de rugosité superficielle d'une taille moyenne de particules non supérieure à 2 pm, cette couche présentant une rugosité microscopique de sa surface externe de telle sorte que chaque millimètre carré de cette surface contient au moins 200.000 particules qui font saillie au-dessus du niveau moyen de cette surface, suivant au moins 30% de leurs diamètres individuels ou suivant 0,2 um, quelle que soit la valeur qui est la moindre.

7. Elément photographique suivant la revendication 1, caractérisé en ce qu'il comprend une couche dorsale ayant une densité optique de transmission maximale d'au moins 0,3 par rapport à la lumière du proche infrarouge, et une couche superieure contenant un agent de rugosité superficielle d'une taille moyenne de particules non supérieure à 2 µm, cette couche présentant une rugosité microscopique de sa surface externe de telle sorte que chaque millimètre carré de cette surface contient au moins 200.000 particules qui font saillie au-dessus du niveau moyen de cette surface, suivant au moins 30% de leurs diamètres individuels ou suivant 0,2 pm, quelle que soit la valeur qui est la moindre.

8. Elément photographie suivant la revendication 1, caractérisé en ce qu'il comprend une couche de substrat antihalo ayant une densité optique de transmission maximale d'au moins 0,3 par rapport à la lumière dans le proche infrarouge, et une couche dorsale ou une couche supérieure contenant un agent de rugosité superficielle d'une taille moyenne de particules non supérieure à 2 µm, cette couche ayant une rugosité microscopique de sa surface externe, de sorte que chaque millimètre carré de cette surface contient au moins 200.000 particules qui font saillie au-dessus du niveau moyen de cette surface suivant au moins 30% de leurs diamètres individuels ou suivant 0,2 pm, quelle que soit la valuer qui est la moindre.

9. Elément photographique suivant la revendication 1, caractérise en ce qu'il comprend une couche supérieure contenant un agent de rugosité superficielle d'une taille moyenne de particules non supérieure à 2 um, cette couche présentant une rugosité microscopique de sa surface externe, de telle sorte que chaque millimètre carré de cette surface contient au moins 200.000 particules qui font saillie au-dessus du niveau moyen de cette surface suivant au moins 30% de leurs diamètres individuels ou suivant 0,2 um, quelle que soit la valeur qui est la moindre, et une couche dorsale contenant un agent de rugosité superficielle d'une taille moyenne de particules non supérieure à 2 pm, cette couche présentant une rugosité microscopique de sa surface externe de telle sorte que chaque millimètre carré de cette surface contient au moins 200.000 particules qui font saillie au-dessus du niveau moyen de cette surface, suivant au moins 30% de leurs diamètres individuels ou suivant 0,2 pm, quelle que soit la valeur qui est la moindre, et éventuellement une couche de substrat contenant un colorant antihalo donnant une sensité optique de transmission maximale d'au moins 0,3 par rapport à la lumière dans le proche infrarouge.

10. Elément photographique suivant la revendication 1, caractérisé en ce qu'il comprend une couche dorsale et/ou une couche supérieure, comprenant un liant contenant des particules d'un indice de réfraction sensiblement plus éléve que celui du liant ayant une taille moyenne de particules inférieure à 5 um, cette ou ces couches étant séparables durant le traitement photographique.

11. Elément photographique suivant la revendication 10, caractérisé en ce qu'il est sensible à un rayonnement dans l'intervalle de longueurs d'onde de 750 à 900 nm.

12. Elément photographique suivant l'une l'une quelconque des revendications 1 à 3 et 5 à 9, caractérisé en ce que les particules de l'agent de rugosité ont une taille moyenne de particule de l'ordre de 0,2 à 2 µm.

13. Elément photographique suivant l'une quelconque des revendications 1 à 3 et 5 à 9, caractérisé en ce que l'agent de rugosité est choisi parmi le polyméthyl méthacrylate et les copolymères d'acide méthacrylique avec du méthacrylate de méthyl ou d'éthyle.

14. Elément photographique suivant la revendication 10, caractérisé en ce que la matière d'un indice de réfraction élevé a une taille moyenne des particules de l'ordre de 0,2 à 3 um.

15. Elément photographique suivant la revendication 14, caractérisé en ce que la matière d'un indice de réfraction élevé est choisi parmi les halogénures d'argent, l'oxyde de zinc et le carbonate de calcium.

16. Procédé d'enrigistrement d'une image pratiquement exempte de franges d'interférence sans contact, qui comprend l'exposition d'une élément photographique suivant l'une quelconque des revendications précédentes en l'absence d'un contact avec d'autres surfaces, à un rayonnement dans le proche infrarouge provenant d'une système de balayage à diode laser, disposé du côté émulsion de l'élément photographique, avec ensuite traitement de cet élément pour développer l'image.
